

# United States Patent Office

2,929,743

Patented Mar. 22, 1960

1

2,929,743

## PROCESS FOR TREATING CELLULOSE MATERIAL WITH THERMOPLASTIC MATERIAL AND PRODUCT THEREOF

Guido Mino and Gamal Eldin Cordahi, Plainfield, N.J., assignors to American Cyanamid Company, New York, N.Y., a corporation of Maine

No Drawing. Application November 8, 1956  
Serial No. 621,015

8 Claims. (Cl. 117—139.5)

This invention relates to the treatment of cellulosic containing textile materials and more preferably cotton containing textile material with a composition comprising as essential components a thermosetting aminoplast resin and a thermoplastic copolymer latex in which the said components are present in critical amounts and in which the thermoplastic copolymer is of critical composition.

The concept of treating cellulosic textile materials with water-soluble aminoplast resins, as for example, methylated methylol melamine resins, is known and described in U.S. Patent No. 2,339,203, and it has also been suggested in the prior art that textile materials including cotton textile materials be impregnated with various thermoplastic materials, among which are polymeric esters of unsaturated aliphatic acids, as for example, polymeric methyl acrylate.

In addition, in U.S. Patent No. 2,536,050, the combination of thermoplastic copolymers and thermosetting resins, have been suggested for use in the treatment of textile materials for purposes of imparting superior crease resistance, abrasion resistance, and the like thereto. While, for the most part, the compositions described in U.S. Patent 2,536,050 are suitable, certain limitations have been found to exist in the textile material which has been so treated.

Among the deficiencies reported from the application of the compositions described in this patent is that the "hand" of the fabric tends to be too stiff and/or too soggy. With respect to this deficiency, its importance is magnified when one considers the adverse effect on sales which results from such a property. Thus, for example, fabric having a stiff and/or soggy hand is generally not acceptable for personal clothing; nor are they desirable for fabrics such as are employed for use as drapery material, slip covers and the like.

Therefore, it is an object of the present invention to provide a thermoplastic composition which, when employed with a thermosetting aminoplast resinous material, may be applied to the cellulosic textile materials so as to impart a soft, full, dry hand to the treated fabric.

It is a further object to provide a thermoplastic composition, which, when employed in connection with a thermosetting aminoplast resinous material, will, in addition to providing the above enumerated effects, enhance the "wash and wear" qualities of the fabric so treated, abrasion resistance, and will be durable to washing and dry cleaning as well as imparting other desirable properties thereto.

These and other objects and advantages will become apparent from the following description of the present invention set forth hereinbelow.

According to the present invention, a process is provided for improving the properties of a cellulosic textile material which comprises impregnating the said textile material with a combination of (1) a heat-curable aminoplast resinous material which is at least partially water-soluble and (2) a substantially water-insoluble thermoplastic copolymer composition that is the product of polymerization of polymerizable monomers, said monomers consisting of a substantially azeotropic mixture of a styrene and a lower alkyl ester of acrylic acid, wherein the

2

alkyl group contains from 1 to 4 carbon atoms. The products of (1) and (2) are employed in weight ratios corresponding to from 2 to 4 parts of the former for each part of the latter. Thereafter, (1) is cured in situ

5 in intimate contact with (2) to a substantially water-insoluble state, the amount of the products of (1) and (2) applied to the textile material being such that the finished textile contains from between 2½ to 20% by weight based on the weight of the dry textile.

10 By "a substantially azeotropic mixture" as the term is used herein, is meant one which will produce a copolymer substantially free of homopolymer, of either of the reacting components or monomers. The ratio of the reactants to produce such copolymers are based on the 15 reactivity of the reacting components or monomers rather than on their molecular weights. Azeotropic mixtures and copolymers are defined more fully in the text "Mechanism of Polymer Reaction" by G. M. Burnett, copyright 1954, at page 249.

20 In the application of the mixed resinous composition, the thermosetting resinous material is used in an amount of from between 2 and 4:1 and preferably about 3.5:1 with respect to the thermoplastic azeotropic copolymer composition.

25 In accordance with the present invention, the water-insoluble thermoplastic compositions are employed in admixture with thermosetting aminoplast resins so as to apply from between 0.5% and 5% of the thermoplastic copolymer and preferably from between 1 and 3% thereof

30 and from between 2 and 15% of the thermosetting aminoplast material and preferably from between 3.5 and 10% thereof, all percentages being based on the dry weight of the textile fabric. Thus, from between 2.5 and 20% of a suitable treating composition may be applied to 35 the fabric, and preferably from between 4.5 and 13% is applied thereto.

The thermosetting aminoplast resin employed with the thermoplastic water-insoluble copolymer must be heat curable and at least partially water soluble. Included

40 in the term "aminoplast resin" by way of example are melamine-formaldehyde reaction products, alkylated melamine-formaldehyde reaction products, guanamine and substituted guanamine-formaldehyde reaction products, including their alkylated derivatives, urea-formaldehyde

45 reaction products, including cyclic ureas, such as ethylene urea, 1,2 and 1,3 propylene urea, and their alkylated derivatives and the like, employed either singly or in combination with one another. The methylol and alkylated methylol derivatives of these compounds may readily be prepared by methods well known to those skilled in the art.

Melamine-formaldehyde reaction products including their alkylated derivatives, are the preferred thermosetting aminoplast resin. These heat-curable reaction

55 products may be used when at least partially soluble in water, though preferably they are substantially completely water soluble, either in the form of a true solution, or as a colloidal dispersion. Examples of melamine-formaldehyde reaction products that may be employed

60 are those which contain one or more methylol groups, more particularly, di, tri, tetra, penta, or hexamethylol melamine, or mixtures thereof.

Such products may be produced in known manner by effecting reaction under neutral or alkaline conditions 65 between melamine and an aqueous solution of formaldehyde in the ratio of 1 mole of the former to from between 2 to 6 moles of the latter. To avoid the formation of the crystalline material, which has lower water solubility and to obtain the amorphous product of higher water solubility, the mass, advantageously, is maintained at a temperature not less than about 70° C. during the reaction. In order to minimize polymerization of the mon-

omer, it is usually desirable to keep the reaction temperature from exceeding about 90° C.

The curable alkylated or alcohol reacted methylol melamine, more particularly, methylated polymethylol melamines, are especially suitable for use in practicing the present invention. They may be prepared, for example, by effecting reaction under acidic conditions, between a polymethylol melamine and a saturated aliphatic alcohol, containing from 1 to 4 carbon atoms in the ratio of 1 mole of the former to from 2 to 6 moles of the latter, depending upon the number of methylol groups in the melamine derivative, and the extent of etherification desired. The reaction is stopped before the product becomes hydrophobic. Alkali is added in an amount at least sufficient to neutralize the reaction mass, after which the mass is dehydrated under vacuum. Advantageously, the methylated methylol melamine, more particularly, polymethoxymethyl melamine, is prepared in the manner such as is disclosed and claimed in U.S. Patent No. 2,529,856.

The thermoplastic copolymer latices of the present invention are produced by reacting in azeotropic quantities lower alkyl esters of acrylic acid wherein the alkyl group has from 1-4 carbon atoms and a styrene. Included in the former group are methyl, ethyl, propyl, isopropyl, butyl, isobutyl, and tertiary butyl acrylates.

Among the styrenes which may be employed are styrene per se, ring-substituted vinyl toluenes, and side-chain substituted styrenes. Examples of the latter two are chlorovinyl toluenes, methylvinyl toluenes (o, m, p),  $\alpha$ -methyl styrene,  $\alpha$ -ethyl styrene and the like.

The thermoplastic copolymer employed in the present invention is produced by copolymerizing substantially an azeotropic mixture of a styrene and a lower alkyl ester of acrylic acid, in which the alkyl substituent contains from 1 to 4 carbon atoms by methods known to those skilled in the art, such as those generally described in application, Serial No. 636,279, filed December 20, 1945, which is now abandoned, and in detail by way of example hereinafter.

Azeotropic compositions of the suitable reactants within the meaning of the present invention can be each calculated from the reactivity ratio of a monomer pair, and then checked experimentally by usual analytical methods as is well known to those skilled in the art.

In this manner, it has been determined that the azeotropic mixture for the styrene-ethyl acrylate copolymer system is 80 parts of styrene and 20 parts of ethyl acrylate by weight in 100 parts of mixture. With respect to the styrene-butyl acrylate copolymer system, in a 100-part mixture, 57 parts are styrene and 43 parts are butyl acrylate which constitutes the azeotropic copolymer composition.

In all of the thermoplastic copolymer compositions contemplated by the present invention, the styrene component is present by weight in amounts significantly in excess of 50% of the total copolymer composition. Thus, in the case of styrene and butyl acrylate, the latter is present as 43% by weight of the copolymer, while in the case of styrene and ethyl acrylate the latter is present as 20% by weight of the mixture.

The components of the thermoplastic copolymer must be present in substantially azeotropic quantities, in order to produce optimum "hand" properties. Thus, in the case of the styrene-ethyl acrylate copolymer, a mixture of exactly 80 parts of the former to 20 parts of the latter is optimum, although an acceptable copolymer mixture can vary slightly. Thus, for example, between 78 and 82 parts of the former to 22 to 18 parts of the latter may be used with acceptable results.

A property of the thermoplastic copolymer of the present invention is that it is water insoluble and must be applied as an emulsion. As used with a thermosetting resin, such as methylated methylol melamine, in which it is frequently highly desirable to employ a metal salt

as a curing catalyst therefor, coagulation of the thermoplastic copolymer often results. This is particularly true when the metal salt catalyst is a salt of heavy metal ions such as magnesium chloride and zinc nitrate. The coagulating effect produced by a normal amount of such salt-curing catalyst may be overcome by using about 2% solids of a non-ionic surface active agent, based on the solids in the thermoplastic copolymer emulsion. This obviates the problem produced by coagulation, provided that the thermoplastic copolymer emulsion is added to the metal salt catalyst which usually is in admixture with the thermosetting resin. Any non-ionic agent is suitable here, as for example, those by the trade names of Triton X 100, the Pluronics, and Deceresol NI Conc. While the amount set forth hereinabove was expressed as 2% solids, the amount necessary is actually controlled by the amount of catalyst employed in the system.

As a process for producing the thermoplastic copolymers, a suitable vessel equipped with an agitator, reflux condenser, graduated dropping funnel, thermometer and heating means is provided, and in it are placed 350 parts of water and 2.5 parts of a non-ionic surface active agent, such as Duponol C, the active component of which has been identified as sodium lauryl sulfonate. The temperature is then raised to about 85° C. and 200 parts of an azeotropic monomer mixture, as for example, 20% (40 parts) of ethyl acrylate, and 80% (160 parts) of styrene by weight is added with continuous stirring, in 10-portion increments, a single portion being added every 15 minutes or so. After each feed period an aliquot addition of ammonium persulfate, initiator and a sodium bicarbonate buffer solution is added.

As an example of a suitable initiator composition, 0.268 part of ammonium persulfate dissolved in 50 parts of water functions in a highly desirable manner. As illustrative of the buffer solution, 0.3 part of sodium carbonate is usually sufficient to effect the necessary buffering action, where proportions of the magnitude set forth hereinabove are employed.

After the addition is completed, the reaction mixture is refluxed with stirring for an additional 30 minutes. Thereafter, the residual monomers are removed by steam distillation, and preferably there is added 16 parts of a non-ionic wetting agent, as for example, Deceresol NI Conc., an alkyl aryl polyether alcohol, and finally the pH is adjusted to 8 with dilute ammonium hydroxide. The percentage of conversion from monomer mixture to polymer composition was approximately 97%.

Employing the general procedure outlined hereinabove, water-insoluble thermoplastic copolymers within the meaning of the present invention may be prepared.

For the application of the thermoplastic copolymer and the thermosetting resin to cellulosic textile materials, a pad bath is made up of a suitable thermosetting resin, as for example, methylated methylol melamine, to which catalyst has been added, and thereafter the thermoplastic copolymer, preferably containing, in addition, a non-ionic surface active agent, is stirred in.

The amount of catalyst employed is usually from between about 1 to 60% and preferably amounts of the order of between 2 and 25% based on the weight of the thermosetting resin which is applied to the fabric. Suitable catalysts within the meaning of the present invention are ammonium salts such as ammonium chloride; amine salts such as trimethylamine hydrochloride; alkanolamine salts such as triethanolamine hydrochloride; and metallic salts such as magnesium chloride and zinc nitrate.

Impregnation on the treatment of the fabric may be carried out in a number of different ways. The fabric may be impregnated, as for example, by soaking, immersion, dipping, spraying, padding, or the like, or other means known to those skilled in the art.

After the application of the resinous composition to the cellulosic textile fabric to be treated, it may be run through suitable squeeze rollers or other means whereby

the desired amount of resin solids may be controlled, as well as excessive free moisture removed therefrom. Thereafter, the fabric may be dried until dry to the touch, as for example, at from 175° F.-250° F. and then cured, as for example, from 3 minutes at 350° F. to 0.5 minute at 450° F. or the fabric may be dried and cured in a single operation, as for example, for from 6 minutes at 290° F. to 1.5 minutes at 450° F.

The following examples are given primarily by way of illustration in order that the present invention may be more fully understood. No details therein should be construed as limitations on the present invention except as they appear in the appended claims. All parts and percentages are by weight unless otherwise designated.

#### EXAMPLE 1

A piece of 80 x 80 cotton was padded through a composition consisting of a thermoplastic copolymer emulsion containing 2 parts of an azeotropic copolymer composition containing 80% styrene-20% ethyl acrylate by weight and .04 parts of a non-ionic surface active agent are mixed with an aqueous solution containing 5 parts of a water-soluble methylated methylol melamine and .6 part of magnesium chloride as a curing catalyst.

The treated material was then run through a squeeze roll adapted to provide a 100% wet pick-up. Thereafter, the fabric was dried 2 minutes at 225° F. and cured at 350° F. for 1.5 minutes.

The following table is for purposes of registering comparisons of the properties of various thermoplastic copolymer latices when used in conjunction with a thermosetting resin and applied to cloth. In all cases, the resins were applied as in Example 1 so as to apply 5 parts of a water-soluble heat-curable methylated methylol melamine as the thermosetting resin and 2 parts of thermoplastic copolymer. The composition of the thermoplastic portion of the resinous compositions are set forth in columns 2 and 3 of the table, according to their content of styrene and ethyl acrylate, respectively, and are generally prepared as described hereinabove.

Table I

COMPARISON OF THE EFFECT ON HAND ON 80 x 80 COTTON

| Resin No. | Composition of Thermoplastic Copolymer, percent |    | 5% Melamine Resin +2% Thermoplastic Copolymer, Hand |      |            |
|-----------|-------------------------------------------------|----|-----------------------------------------------------|------|------------|
|           | Styrene                                         | EA | Soft                                                | Full | Dry        |
| 1-----    | 10                                              | 90 | soft                                                | full | sl. soggy. |
| 2-----    | 50                                              | 50 | stiff                                               | full | soggy.     |
| 3-----    | 65                                              | 35 | firm                                                | full | sl. soggy. |
| 4-----    | 80                                              | 20 | soft                                                | full | dry.       |
| 5-----    | 90                                              | 10 | soft                                                | thin | dry.       |

<sup>1</sup> Azeotropic mixture.

It will be observed that in all cases where the amounts of ethyl acrylate and styrene employed in making the thermoplastic composition were not present in azeotropic amounts, the treated cotton was deficient in that the hand tended to be soggy or thin.

This is believed to be produced either by the presence of homopolymer of an acrylate or homopolymer of a styrene. Thus when the copolymer composition is not azeotropic and homopolymer of a styrene is present, the hand tends to be thin and dry. When not an azeotropic copolymer composition, and a homopolymer of an acrylate is present, the hand tends to be full, but soggy, or what is sometimes termed a "dead hand."

Among other advantages of the present process are

15 the durability to dry cleaning and the durability to washing of the finish applied. Table II, set forth hereinbelow, points out these advantages by comparative test results. In determining durability of a particular finish to dry cleaning, tentative test method 25-52, at page 76 of the 20 A.A.T.C.C. yearbook of 1955, was generally employed. In this method, swatches of the treated fabric are placed in a laundrometer in jars containing Varsol No. 2, a Stoddard Solvent. The jars are run 25 minutes at 80° F. and thereafter the samples are removed and centrifuged 25 dry. The fabrics are then steam pressed, conditioned, and evaluated for hand. (This test differs from 25-52 in that no soap is employed. The soap is difficult to remove from the fabric and could affect hand, and since durability to washing is also determined, the omission of the 30 soap is considered a valid deletion in this test.)

In determining the durability to washing of the finish, swatches of a treated fabric are washed in an agitator washer for 45 minutes in a 0.1% soap and a 0.1% soda ash at 160° F. The fabrics are then thoroughly rinsed 35 in water at 160° F. (three 5-minute washes) centrifuged, and pressed on a flat bed ironer at 325° F. for 30 seconds. The fabrics were then conditioned and evaluated for hand. This procedure is similar to the standard test method 36-54, page 56 of the 1955 A.A.T.C.C. yearbook, except that larger swatches are employed, which necessitates an agitator wash instead of the laundrometer. The wash employed also necessitated the modification of the soap concentrations.

In Table II, all of the applications were made in a 45 manner similar to that set forth in Example 1 hereinabove.

It will thus be seen according to Table II that where the resin treatment employed contains an azeotropic copolymer composition of a lower alkyl acrylate and styrene, the hand of the treated fabric is soft, full and dry. 50 The durability of the hand imparted by the azeotropic copolymer and melamine resin is of the same order as obtained with other thermoplastic copolymers and melamine resin compositions. However, the appearance of fabric treated with the azeotropic copolymer and melamine resin is enhanced after washing compared to the 55

Table II

| Resins           | Composition of Thermoplastic Copolymer, percent |                |                | 5% Melamine Resin +2% Thermoplastic Copolymer Applied to 80 x 80 Cotton, Hand |                  |                  |                          |
|------------------|-------------------------------------------------|----------------|----------------|-------------------------------------------------------------------------------|------------------|------------------|--------------------------|
|                  | Styrene                                         | Ethyl Acrylate | Butyl Acrylate | Initial                                                                       | Washed           | Dry Cleaning     | Wash and Wear—Appearance |
| 1-----           | 10                                              | 90             |                | SO; F; SG-----                                                                | SO; F; SG-----   | SO; F; SG-----   | Poor.                    |
| 2-----           | 50                                              | 50             |                | ST; F; SG-----                                                                | ST; F; SG-----   | ExST; F; SG----- | Fair.                    |
| 3-----           | 65                                              | 35             |                | SO; F; SLSG-----                                                              | SO; F; SLSG----- | SO; F; SLSG----- | Fair.                    |
| 4-----           | 1 80                                            | 1 20           |                | SO; F; D-----                                                                 | SO; F; D-----    | SO; F; D-----    | Good.                    |
| 5-----           | 90                                              | 10             |                | SO; T; D-----                                                                 | SO; T; D-----    | SO; T; D-----    | Fair.                    |
| 6-----           | 80                                              |                | 20             | SO; T; D-----                                                                 | SO; T; D-----    | SO; T; D-----    | Fair.                    |
| 7-----           | 1 57                                            |                | 1 43           | SO; F; D-----                                                                 | SO; F; D-----    | FI; F; D-----    | Good.                    |
| Untreated Fabric |                                                 |                |                | SO; T; D-----                                                                 | SO; T; D-----    | SO; T; D-----    | Poor.                    |

<sup>1</sup> Legend: Azeotropic compositions.

Code: D=dry; EX=extra; F=full; FI=firm; SG=soggy; SL=slight; SO=soft; ST=stiff; T=thin.

7  
other combinations and may be said to have the characteristics of a wash and wear finish.

Although this invention has been described with particular reference to the treatment of cotton, specifically cotton fabrics, the treatment herein described may also be applied to other textiles which are composed substantially or mainly of cellulose or regenerated cellulose, for example, linen, hemp, jute, ramie, sisal, cellulose acetate rayons, cellulose acetate butyrate rayons, saponified acetate rayons, viscose rayons, cuprammonium rayons, ethyl cellulose, and mixtures thereof, with each other or with cotton.

The term "textile" and "textile material" as used generally herein and in the appended claims, include within their meaning filaments, fibers, threads, yarns, twisted yarns, etc. as such, or in woven, non-woven or otherwise formed fabrics, sheets, cloths, and the like.

In addition to the essential components of the treating composition set forth hereinabove, namely, the thermoplastic copolymer, the thermosetting resin and the acid acting curing catalyst for the thermosetting resin, other additives which are not inconsistent and do not destroy the effect of the essential components of the present invention may be added therewith, as for example, softeners, antistatic agent, fillers, pigments, dyes, and the like, may be incorporated into the bath solution and applied simultaneously with the resin composition of the present invention.

The impregnated cotton or other cellulosic textile material of this invention is also resistant to shrinkage, as well as to wear and abrasion. The finish is durable and is not removed by washing in water and, in addition, is durable to dry cleaning, as noted in Table II above. The hand may be varied slightly, for example, by varying the kind and amount of thermoplastic modifier employed and/or the kind and amount of thermosetting resin within the limits set forth hereinabove.

We claim:

1. A process of improving the properties of cellulosic textile material which comprises impregnating the said textile material by imparting a soft, full, dry hand thereto, which is durable to dry cleaning and laundering, with a combination of (1) a partially water-soluble heat-curable synthetic aminoplast resin and (2) a substantially water-insoluble thermoplastic copolymer composition, the product of polymerization of polymerizable monomers, said polymerizable monomers consisting of an azeotropic mixture of a styrene and a lower alkyl ester of acrylic acid, wherein the styrene is present in an amount by weight in excess of 50% of the copolymer composition, and wherein the alkyl group contains from 1 to 4 carbon atoms, the products of (1) and (2) being employed in weight ratios corresponding to from 2 to 4 parts of the former for each part of the latter, and curing in situ (1) in intimate contact with (2) to a substantially water-insoluble state, the amount of the product of (1) and (2) applied to said textile material being such that the finished textile contains from 2.5 to 20% by weight of the dry textile material.

2. A process of improving the properties of cellulosic textile material which comprises impregnating the said textile material by imparting a soft, full, dry hand thereto, which is durable to dry cleaning and laundering, with

5 a combination of (1) a partially water-soluble heat-curable reaction product of ingredients comprising melamine and formaldehyde and (2) a substantially water-insoluble thermoplastic copolymer composition, the product of polymerization of polymerizable monomers, said polymerizable monomers consisting of an azeotropic mixture of a styrene and a lower alkyl ester of acrylic acid, wherein the styrene is present in an amount by weight in excess of 50% of the copolymer composition, and wherein the alkyl group contains from 1 to 4 carbon atoms, the products of (1) and (2) being employed in weight ratios corresponding to from 2 to 4 parts of the former for each part of the latter, and curing in situ (1) in intimate contact with (2) to a substantially water-insoluble state, the amount of the product of (1) and (2) applied to said textile material being such that the finished textile contains from 2.5 to 20% by weight of the dry textile material.

3. A process according to claim 2 wherein the azeotropic thermoplastic copolymer is comprised of styrene and ethyl acrylate.

4. A process according to claim 2 wherein the azeotropic thermoplastic copolymer is comprised of styrene and butyl acrylate.

5. A process according to claim 2 wherein the azeotropic thermoplastic copolymer is comprised of methylvinyl toluene and ethyl acrylate.

6. A process according to claim 2 wherein the azeotropic thermoplastic copolymer is comprised of methylvinyl toluene and butyl acrylate.

7. A process according to claim 2 wherein the weight ratio between the products of (1) and (2) is 3.5 parts of the former to 1 part of the latter, and wherein the amount of the products of (1) and (2) applied to the textile material is from between 4.5 and 13% based on the weight of the dry textile material.

8. A cellulosic fabric material having a soft, full, dry hand which is durable to dry cleaning and laundering, which is impregnated with from 2½ to 20% by weight of the dry fabric material of a combination of (1) a substantially water-insoluble cured product which prior to curing is an at least partially water-soluble curable synthetic aminoplast resin and (2) an azeotropic thermoplastic copolymer composition that is the product of polymerization of polymerizable monomers consisting of an azeotropic mixture of a styrene and a lower alkyl ester of acrylic acid, wherein the styrene is present in an amount by weight in excess of 50% of the copolymer composition, and wherein the alkyl group contains from 1 to 4 carbon atoms and in which the products of (1) and (2) have been employed in weight ratios corresponding to from 2 to 4 parts of the former for 1 part of the latter, and in which (1) has been cured in situ in intimate contact with (2) to said substantially water-insoluble state.

55 References Cited in the file of this patent

UNITED STATES PATENTS

|           |                    |                |
|-----------|--------------------|----------------|
| 2,054,131 | Kollek             | Sept. 15, 1936 |
| 2,123,599 | Fikentscher et al. | July 12, 1938  |
| 2,140,048 | Fikentscher et al. | Dec. 13, 1938  |
| 2,563,898 | Wilson et al.      | Aug. 14, 1951  |
| 2,823,142 | Sumner et al.      | Feb. 11, 1958  |